

Oct. 2, 1923.

1,469,566

J. WEISHÄUPL

METHOD OF MANUFACTURING TURBINE ROTORS

Filed Dec. 11, 1922

Fig. 1



Fig. 2



Fig. 3



Fig. 4



Inventor:  
Joseph Weishäupl  
By Henry Ott atty.

## UNITED STATES PATENT OFFICE.

JOSEPH WEISHÄUPL, OF ZURICH, SWITZERLAND, ASSIGNOR TO THE FIRM AKTIEN-  
GESELLSCHAFT DER MASCHINENFABRIKEN ESCHER WYSS & CIE, OF ZURICH,  
SWITZERLAND.

## METHOD OF MANUFACTURING TURBINE ROTORS.

Application filed December 11, 1922. Serial No. 606,152.

To all whom it may concern:

Be it known that I, JOSEPH WEISHÄUPL, a citizen of the Republic of Switzerland, residing at Zurich, Switzerland, have invented certain new and useful Improvements in Methods of Manufacturing Turbine Rotors, of which the following is a specification, reference being had therein to the accompanying drawing.

In order to obtain high efficiencies with rotary engines, especially steam turbines and gas turbines, it is frequently necessary to adopt high speeds. This, for instance, is the case with steam turbines of small output when a low steam consumption is desired. With high speed turbines the rotor wheels show comparatively large dimensions in the parts forming the boss and they have a correspondingly large weight when the rotor wheels are manufactured in the known manner, i. e., when every rotor wheel is manufactured separately and the rotor wheels are mounted singly on a shaft. The large weights of the rotor wheels require, however, a comparatively thick shaft which in its turn influences unfavourably the steam consumption and the costs for manufacturing the turbine. With steam turbines of small output it is therefore endeavoured to keep the shaft and the rotor wheels as light as possible. The smallest dimensions and the smallest weights as well as the greatest strength are obtained when the rotor wheels and the shaft are forged from one piece. Rotors of this type are known and they are manufactured by forging the whole rotor out of one block, to which is given at first the shape corresponding to the outer configuration of the rotor, whereupon the definite shape is given to the rotor by turning off the material present between the single discs, the shape of the discs conforming to discs of uniform strength.

In order to obtain a homogeneous material for the parts of the shafts between adjacent discs, it is necessary in this case to forge also the material between the discs down to the diameter of the shaft. With the known processes this is, however, not possible as the forging down of the material between the discs of the block would result in an exceedingly large increase of

the distance between the discs, which increase is obviously inadmissible. 55

The novel process consists in that the material between the discs is not forged down to the diameter of the shaft but is by steps rough turned off on a lathe. After the first step of rough turning the remaining material between the discs is forged and thereby made homogeneous, whereupon further material is removed on a lathe during the next step, a further forging and homogenizing of the remaining material being effected and so on until the forging of the rotor is finished and the latter is ready to be finally machined on the lathe. Every step of the forging of the material between the discs causes a small lengthening of the shaft but this lengthening may be compensated by immediately pressing both ends of the forging towards each other while it is still hot.

The novel process shall now be explained 75 with reference to the accompanying drawing. The figures illustrate several rotors manufactured according to the novel process, and in which:

Fig. 1 is a view of a rotor, the adjoining shaft pieces being fixed by means of screws to the rotor proper, 80

Fig. 2 is a view of a rotor which is subdivided at two intermediate discs, and

Fig. 3 is a view of a rotor which is only 85 subdivided at the middle disc.

Fig. 4 is a view of a rotor which forms one integral piece with the adjoining shaft pieces.

When a rotor of the type illustrated in Fig. 1 is to be manufactured according to the present process, to a block 1 will be given the shape indicated in Fig. 1 in dotted lines which shape corresponds to the outer configuration of the rotor. From this forged block 1 part of the material is hereupon rough turned off on a lathe, for instance, up to the chain-dotted line 11 whereby annular recesses are formed. Then the material in this recess can be forged to be made homogeneous. Through this forging process the distance between the discs is somewhat increased which increase may be counteracted by pressing both ends of the forging in the axial direction towards 100 each other. By a second step in the process 105

the material is rough turned off on a lathe up to the chain-dotted line 12, whereupon the forging and homogenizing takes place. According to the size of the block further similar steps in the process may be necessary until the rotor has the shape shown by the chain-dotted line 13. With rotors having small outside diameters and therefore a small depth of the recesses it is possible to employ only one step i. e. to rough turn off the material only once and thereafter to homogenize by forging.

In this manner the material on the sides of the discs as well as the part of the shaft between the discs is made homogeneous so that a rotor forged in this manner will respond to the highest requirements.

The rotor may be subdivided into single parts as is shown in Figs. 2 and 3, in which the rotor is subdivided twice at the discs 8, 9 and once at the disc 10 respectively; however, the whole rotor together with the outer parts of the shafts may be made from one single forging, as is shown in Fig. 4.

25 I claim:

1. The process of manufacturing rotors for turbines, the rotor wheels or discs of which are integral with the appertaining part of the shaft, which consists in treating blocks forged to a determined outer configuration so as to form recesses in said

block corresponding to intermediate spaces to be provided between the rotor discs, and subjecting the material between the discs of the rotor to a homogenizing action during said treatment.

2. The process of manufacturing rotors for turbines, the rotor wheels or discs of which are integral with the appertaining part of the shaft, which consists in rough turning off from a block forged to a determined outer configuration material to form recesses separating the discs of the rotor, and homogenizing the inner material remaining between the discs to obtain the recesses separating the discs of the rotor.

3. The process of manufacturing rotors for turbines, the rotor wheels or discs of which are integral with the appertaining part of the shaft, which consists in rough turning off from a block forged to a determined outer configuration material to form recesses separating the discs of the rotor, homogenizing the inner material remaining between the discs, and alternately repeating the rough turning and the homogenizing step until recesses of the required depth are obtained between the discs.

In testimony whereof I affix my signature.

JOSEPH WEISHÄUPL